

April 20, 1937.

LE ROY G. STORY

2,077,781

LUBRICATING OIL

Filed Aug. 1, 1934



Le Roy G. Story  
INVENTOR

BY R. J. Dearborn

his ATTORNEY

## UNITED STATES PATENT OFFICE

2,077,781

## LUBRICATING OIL

LeRoy G. Story, Glenham, N. Y., assignor to The  
Texas Company, New York, N. Y., a corporation  
of Delaware

Application August 1, 1934, Serial No. 737,961

3 Claims. (Cl. 196—78)

This invention relates to the manufacture of lubricating oils, and particularly synthetic lubricating oils, as well as blends of petroleum lubricating oils with such synthetic oils to provide oils 5 of improved character having an increased viscosity index.

In the production of high grade lubricating oils, it is well known that a relatively small change in the viscosity of the oil between temperatures of 10 say 100° F. and 210° F., is desirable. In other words, it is advantageous for the oil to have a relatively flat viscosity-temperature curve, which means that the oil has a high viscosity index as defined by Dean and Davis in their article in 15 Chemical and Metallurgical Engineering, vol. 36, page 618. Improvement in lubricating oils has heretofore been accomplished by refining, as by the use of selective solvents which are effective in extracting or separating naphthenic constituents 20 from paraffinic constituents, thereby producing a resulting raffinate of increased viscosity index. This procedure involves expensive processing, and results in a reduced yield of finished oil.

The advantage of low pour point of a lubricating oil has long been recognized. Paraffin base 25 and Mid-Continent lubricating oils have been subjected to dewaxing in order to reduce the pour point thereof. However, substantially complete removal of wax from such oils results in a lowering 30 in viscosity index.

The present invention relates to the increase 35 in viscosity index of naphthene base or paraffin base lubricating oils, by blending therewith a proportion of a material which is active to increase the viscosity index without objectionably affecting other desirable properties thereof. The invention 40 also relates to the preparation of a synthetic lubricating oil of high viscosity index which is suitable for the above purpose, and which is the oily condensation product obtained by condensing in the presence of a metallic halide condensation 45 catalyst the chlorinated product of a cracked waxy hydrocarbon material.

U. S. Patent No. 1,955,260, dated April 17, 1934, 50 discloses the production of a synthetic lubricating oil by cracking a waxy hydrocarbon material, and then condensing the cracked product with a catalyst such as anhydrous aluminum chloride. In co-pending application, Serial No. 732,091, filed 55 June 23, 1934, a synthetic lubricating oil is produced by chlorinating a waxy hydrocarbon, and then condensing the chlorinated product in the presence of a condensation catalyst such as anhydrous aluminum chloride. Each of these methods is subject to practical limitations in the

quantity of yield and quality of product produced, because the cracking or the chlorination step can only be carried to an intermediate reaction stage in practical operation. Consequently, a comparatively lower yield of product which is inferior 5 to that of the present invention is obtained. The present invention combines both the pre-cracking and pre-chlorination steps prior to condensation, with the result that the effect is cumulative, and higher yields of a product of superior character 10 are obtained.

In accordance with the present invention a waxy hydrocarbon, such as paraffin wax, petroleum, wax tailings, slack wax, as well as heavy 15 oils containing wax and consisting essentially of straight chain hydrocarbons, are utilized as starting materials. For purposes of description, each of the above materials is hereinafter designated in the description and claims as a "waxy hydrocarbon material". The high boiling straight chain 20 hydrocarbon material is first subjected to mild cracking to produce a large yield of partially cracked high boiling hydrocarbons and a small amount of tar and low boiling products. This cracking operation may be carried out under va- 25 por phase conditions, preferably under low pressures such as atmospheric to about 100 lbs. per square inch or below, and at temperatures between about 750° and 1100° F. A heavy distillate oil is obtained from the cracked products by fractiona- 30 tion.

The cracked product, such as the distillate oil, is then subjected to chlorination, as by passing chlorine through the material at slightly elevated 35 temperatures. The chlorination product is then condensed in the presence of a metallic halide condensation catalyst, such as anhydrous aluminum chloride. A heavy synthetic lubricating oil of high viscosity index, generally well in excess of 100, is then separated from the condensation 40 product. This oil may be used alone as a lubricating oil of superior or special character. Preferably, the synthetic oil is blended with a petroleum lubricating oil in order to improve the character of the latter. The proportions in which 45 the several oils may be blended vary widely, but proportions of about 10-50% of the synthetic oil to 90-50% of a petroleum lubricating oil give very satisfactory results.

Referring to the accompanying drawing, a flow 50 sheet of the process of the present invention is illustrated. This is hereinafter described in connection with a specific example falling within the scope of the invention. A paraffin wax is passed from a source of supply 10 to a cracking still 11 55

where it is primarily vaporized and the vapors heated at atmospheric pressure to a temperature of about 800°-900° F. to effect cracking. The cracked vapors are fractionated in a fractionating tower 12, where lighter vapors are removed overhead through suitable condensers to receiving tank 13, and a heavier distillate oil containing a substantial proportion of unsaturated hydrocarbons is removed as a side stream 10 to receiving tank 14. The residue, which is a tarry material, is passed to tank 15.

The distillate oil is supplied from tank 14 to a chlorinating vessel 17, to which chlorine gas is supplied from drum 18. The oil in the chlorinator 15 is preferably maintained at about 70°-25° F., and is agitated during the time that a stream of chlorine gas is passed therethrough. For example, a proportion of about 10-12% chlorine on the weight of the oil may be employed. This 20 serves to form chlorine substitution products of the uncracked and mildly cracked paraffins and addition products of a portion of the unsaturated hydrocarbons.

The chlorinated material is then passed to a 25 condensation vat 20, to which anhydrous aluminum chloride is supplied from bin 21. The oil is preferably maintained at a temperature slightly above the melting point which may range from about 50°-125° F. and is agitated during 30 the condensation treatment, which may be continued for about 18-24 hours. A proportion of about 3-5% of anhydrous aluminum chloride may be employed. The condensation product is then passed to a settling tank 22 where the aluminum 35 sludge is separated and passed to receiving tank 23 from where it may be returned for reuse in the condensation reaction. The resulting oil is passed to storage 24, and is preferably contact filtered in the presence of acid treated clay in 40 the treating tank 25. The oil of improved color and free from suspended impurities is then distilled in a vacuum still 26 to remove lighter products which are collected in receiving tank 27, and to obtain a heavy synthetic oil of high 45 viscosity index which is passed to storage tank 28. Residuum from the vacuum still is discharged to receiver 29. An oil of lubricating character and having a viscosity index of about 100-150 may thus be obtained.

50 Where this oil is to be blended with a petroleum lubricating oil, this is accomplished by introducing predetermined proportions of the synthetic oil from storage 28, and a petroleum lubricating oil from storage 30, into a blending tank 55 31, from which the blended oils are discharged to an oil storage 32 for distribution or further treatment.

While anhydrous aluminum chloride constitutes a very satisfactory condensation catalyst for the

production of the above synthetic lubricating oil, it is to be understood that other metallic halide condensation catalysts of the Friedel-Craft type can be employed, such for example, as the chlorides or other halides of cobalt, manganese, iron, 5 boron, nickel, zinc, antimony, cadmium, tin and the like.

Obviously many modifications and variations of the invention, as hereinbefore set forth, may be made without departing from the spirit and 10 scope thereof, and therefore only such limitations should be imposed as are indicated in the appended claims.

I claim:

1. The method of producing a synthetic lubricating oil which comprises mildly cracking a waxy hydrocarbon material containing primarily saturated hydrocarbons at temperatures within the range of 750-1100° F. and at pressures below 100 pounds per square inch to produce a product 20 containing a substantial proportion of unsaturated hydrocarbons, separating a heavy distillate oil containing a substantial proportion of unsaturated hydrocarbons from the cracked product, chlorinating the heavy distillate oil by passing chlorine therethrough at slightly elevated temperatures to produce substitution compounds of saturated hydrocarbons remaining in the distillate oil separated from the cracked product, condensing the chlorinated oil in the presence of 25 a metallic halide condensation catalyst at temperatures within the range of 50-125° F. for about 18-24 hours, and separating a synthetic lubricating oil of high viscosity index from the condensation product. 30

2. The method of producing a synthetic lubricating oil which comprises mildly cracking a waxy hydrocarbon material containing primarily saturated hydrocarbons to produce a product containing a substantial proportion of unsaturated hydrocarbons, chlorinating the cracked product to produce substitution compounds of saturated hydrocarbons remaining in the cracked product, and then condensing the chlorinated cracked product in the presence of a metallic 40 halide condensation catalyst to obtain a lubricating oil. 45

3. The method of producing a synthetic lubricating oil which comprises mildly cracking paraffin wax to produce a product containing a substantial proportion of unsaturated hydrocarbons, chlorinating the cracked product to produce substitution compounds of saturated hydrocarbons remaining in the cracked product, and then condensing the chlorinated cracked product in the presence of aluminum chloride to obtain a lubricating oil. 55

LE ROY G. STORY.